

## UNITED STATES PATENT OFFICE

MORITZ L. MUELLER, OF SEATTLE, WASHINGTON, ASSIGNOR TO GENERAL DRY KILN COMPANY, OF PORTLAND, OREGON, A CORPORATION

## METHOD OF DRYING LUMBER

No Drawing. Original application filed November 10, 1928, Serial No. 318,594. Divided and this application filed July 3, 1929. Serial No. 375,798.

This invention relates to a method of drying lumber, and the present application is a division of my co-pending application, Serial No. 318,594, filed November 10th, 1928.

5 The parent application aforesaid relates to the use of centrifugal force, in the drying of lumber, and particularly to the use of centrifugal force in conjunction with other natural forces.

10 The present application is devoted to the treatment of lumber under the influence of a plurality of forces applied seriatim. More particularly, the invention relates to the drying of lumber under the influence of centrifugal force, and the subsequent treatment 15 of the lumber with heat or vacuum, or both, and either simultaneously or separately applied.

Under most of the lumber drying systems 20 with which I am familiar, the lumber has been placed in drying kilns, and kept there long enough to remove substantially all of the free water, and as much of the combined water or moisture as possible. It is comparatively easy to get rid of the free water, but not so easy to get rid of the combined water. Under the present invention, it is proposed to very expeditiously get rid of the free 25 water by centrifuging, and thereafter resort 30 to the slower and more expensive removal of the combined water, by other means.

By virtue of this method, the time required 35 for the complete drying of the lumber and the removal of both the free and combined water, is materially reduced. Further, the present method improves the quality of the lumber output, because it insures that all of the lumber that goes into the drying kiln 40 will be in a substantially uniform condition insofar as its degree of dryness is concerned. The initial centrifuging brings the whole mass of lumber to be dried to a substantially uniform degree of dryness before it is subjected to additional steps for the removal of 45 the combined water. If these additional steps are to be carried out in an ordinary drying kiln, under the influence of heat, or a vacuum, or heat and vacuum, the lumber 50 goes into such kiln with all of its constituent

parts of a substantially uniform degree of dryness, as hereinbefore described.

As is set forth in my copending application aforesaid, when heat is applied to liquids in wood, it causes an increase in repulsive efforts of the individual molecules with the result that a pressure greater than the surrounding atmospheric pressure is created. Continued far enough, the liquid boils and creates the equivalent of steam pressure. 55 When the vapor pressure in the wood becomes higher than the surrounding atmospheric pressure, the liquids now in a gaseous or liquid form, travel from the interior of the wood to the surface and in a gaseous form 60 leave the surface when sufficiently repelled, or otherwise actuated.

When the moisture (liquid) content of the outside portion of a piece of wood becomes 65 lower than the inside portion, capillary attraction endeavors to effect an equalization of liquid content, with the result that liquids travel from the wetter portions to the drier portions, through the cell walls of the wood. The cell walls permit this travel 70 through the action of osmotic laws, which operate on many cellular structures including wood.

The lumber driers now in general use are 75 designed to set these two natural forces into action. Such driers may be divided into two classes, i. e. "atmospheric pressure driers," and "vacuum driers."

The action and result in the case of an atmospheric pressure drier is as follows: The 80 lumber is piled in such a way that the various units (boards) are separated so as to expose their surfaces to the surrounding atmosphere; the atmosphere is then heated to a temperature above that of the wood and the 85 heat from the air is transmitted to the solid and liquid portions of the wood. This kinetic (heat) energy increases the vapor pressure of the wood liquids, which tends to force their gaseous product out of the wood. In addition, the heated atmosphere surrounding the 90 wood dries the outer fibres of the same, causing the outer portions of the wood to be drier than the inner portion thereof, with the 95 result that the liquids from the interior of 100

the wood travel to the surface, under capillary attraction, osmosis and from the increased interior vapor pressure. As the surrounding atmosphere receives moisture from the wood by its absorption of these gaseous vapors, it tends to lose its absorbing power and become saturated. To prevent the termination of the evaporative action of the atmosphere by saturation, which would stop capillary movement, the surrounding atmosphere is moved continuously so that the surface of the wood is constantly bathed in an atmosphere capable of maintaining the outer portions of the wood in a drier state than the inner portions thereof. During such movement of the atmosphere, it is suitably conditioned with respect to temperature, humidity, etc., to suit the particular conditions existing at the moment.

The operation and result in the case of "vacuum type driers" is as follows: The lumber is open piled in an airtight chamber, and the atmosphere is extracted from said chamber until conditions therein approach a vacuum. Under this reduction of atmospheric pressure, the force of vapor pressure, in its relation to surrounding pressure, is greater at the same temperature than under normal temperature pressure, and, in addition, the boiling point occurs at lower temperatures. As a result, the liquids in the wood vaporize and are forced (drawn) from the wood into the lower pressures of the surrounding atmosphere. Since the exposed surfaces of the wood may have their moisture removed faster than it comes from the inside portions of the material, capillary attraction usually assists in the transfer of the wood liquid. Driers of this type are usually operated at a temperature equal to, or above, the boiling point of the wood liquids, which results in the boiling off (converting moisture into vapor, transferring it through the wood as vapor, and removing it as vapor) the liquids in the wood. An investigation and review of the many lumber driers designed and in use throughout this country shows that the above described principles are exclusively used, and that differences in design lie in the methods of moving and conditioning the atmosphere within said driers in an endeavor to secure more positive and effective results, from the above described natural forces.

In carrying out the invention, I revolve or swing the pieces of wood at a high speed about a central point. The specific apparatus employed is not of the essence of the invention. It is common in the drying art to employ revolving wheels or cages within which material is placed and the water driven therefrom by the action of centrifugal force when said cages or wheels are rotated at high speed. Devices of this character may be employed and the lumber may be loaded therein in any suitable way. I, preferably, load it with its

width parallel to the radii of the wheel or cage, and with its length parallel to the axis about which the structure is revolved.

The described centrifuging of the lumber is continued until all of the easily removed free water has been thrown from the lumber, and the moisture dissipated from the edges of said lumber. Where the lumber is loaded with its width parallel to the radii of the wheel or cage, it follows that the entrained free water need travel only a distance equal to the width of the board. Liquids in wood are located in two parts of the wood cells, part in the cavities inside of the individual cells, called "free water" and part in physical combination with the cell walls proper, called "combined water." Wood does not shrink with the removal of "free water" but does shrink with the removal of the "combined water." Centrifugal force acts freely on the free water, but to a very limited extent on the combined water. Applying centrifugal force to a group of wood pieces having a variety of different initial moisture percentages to start with, will remove the free water from each until it is gone and result in equalizing the moisture content of all at a point approximating that where all free water has been removed but no combined water. Consequently, there is no shrinkage.

The use of the centrifugal force in the manner described for initially removing the free water yields very important economical results upon a commercial scale.

Owing to extremes of moisture content in any one group of lumber which in commercial practice is gathered into a chamber for being dried together, the control of the osmotic forces becomes uncertain and difficult. Wet groups of pieces enter stages during the drying process when osmotic forces should be stimulated or retarded to secure best results, at different times than drier groups, making it impossible for the process to be administered to produce the most efficient effect on all. This is directly due to the fact that osmotic forces effect both "free" water and "combined" water, making it possible for parts of a board or group of boards, to shrink while other parts of the same board or adjoining boards are still too wet to shrink. The result of this condition is the production of strains in the wood causing it to become unsuitable for its use, or to be sold at a lower price than normal, if allowed to materialize and causing an inefficient and slow application of the process, if guarded against.

After the lumber has been brought to a substantially uniform condition as to its dryness, by the removal of the free water, it is subjected to the action of heat or sub-atmospheric pressure, or to sub-atmospheric pressure in the presence of heat. The removal of the free water quickly and, consequently, cheaply, renders the whole process extremely

economical, because, with the free water removed, the combined water can more readily respond to the action of the heat and/or, vacuum, than would be the case if the free water were still present.

5 Further, the amount of combined water to be removed is so very small in comparison with the amount of free water to be removed that, with the time required for the removal of the free water eliminated, the remaining time required for the removal of the combined water is so short that the lumber can be very expeditiously brought to the desired dry state.

10 15 Further, it is the free water that is principally responsible for wide variations in conditions of lumber at the time that it is placed in a drying kiln, and it is the uneven drying, with the resultant checking and cracking that 20 is chiefly responsible for the degraded condition found in some lumber products. The method of the present invention will go a long way toward correcting these conditions.

Having described my invention, what 25 claim is:

1. The hereindescribed method of drying lumber, which consists of subjecting the same to the action of centrifugal force until the free water is removed therefrom, and thereafter subjecting the same to the action of heat for the removal of the combined water.

2. The hereindescribed method of drying lumber, which consists of subjecting a multiplicity of pieces of lumber having moisture 35 contents of varying degrees to the action of centrifugal force for the removal of the free water and to bring all of said pieces of lumber to substantially the same condition of dryness, and thereafter removing the combined water by subjecting the lumber to the action of heat.

3. The hereindescribed method of drying lumber, which consists of subjecting a multiplicity of pieces of lumber having moisture 45 contents of varying degrees to the action of centrifugal force for the removal of the free water and to bring all of said pieces of lumber to substantially the same condition of dryness, and thereafter removing the combined water by subjecting the lumber to the action of heat, in a partial vacuum.

4. The hereindescribed method of drying lumber, which consists of subjecting a multiplicity of pieces of lumber having moisture 55 contents of varying degrees to the action of centrifugal force for the removal of the free water and to bring all of said pieces of lumber to substantially the same condition of dryness, and thereafter removing the combined water by subjecting the lumber to the action of a body of heated air.

5. The hereindescribed method of drying lumber, which consists of subjecting a multiplicity of pieces of lumber having moisture 65 contents of varying degrees to the action of

centrifugal force for the removal of the free water and to bring all of said pieces of lumber to substantially the same condition of dryness, and thereafter removing the combined water by subjecting the lumber to the action of a body of heated air in a partial vacuum.

6. The hereindescribed method of drying lumber, which consists of subjecting a multiplicity of pieces of lumber having moisture 70 contents of varying degrees to the action of centrifugal force for the removal of the free water and to bring all of said pieces of lumber to substantially the same condition of dryness, and thereafter removing the combined water by subjecting the lumber to the action of sub-atmospheric pressure.

7. The hereindescribed method of drying lumber, which consists of centrifuging the same in a direction across the lumber until the free water is removed and thereafter subjecting the lumber to heat, to remove the combined water.

8. The hereindescribed method of drying lumber, which consists of centrifuging the same in a direction transversely of the pieces of lumber until the free water is removed and the various pieces of lumber are brought to substantially the same condition of dryness, and thereafter subjecting the said 95 pieces of lumber to the action of heat, to complete the drying by the removal of the combined water.

9. The hereindescribed method of drying lumber, which consists of centrifuging the same in a direction transversely of the pieces of lumber until the free water is removed and the various pieces of lumber are brought to substantially the same condition of dryness, and thereafter subjecting the said pieces of lumber to the action of a vacuum.

10. The hereindescribed method of drying lumber, which consists of centrifuging the same in a direction transversely of the pieces of lumber until the free water is removed and the various pieces of lumber are brought to substantially the same condition of dryness, and thereafter subjecting the said pieces of lumber to the action of heat in the presence of sub-normal pressure.

In testimony whereof I affix my signature.  
MORITZ L. MUELLER.

120

125

130